

L. F. HAWLEY.

## PROCESS FOR PRODUCING DENSE CHARCOAL.

APPLICATION FILED APR. 3, 1919.

1,369,428.

Patented Feb. 22, 1921.



# UNITED STATES PATENT OFFICE.

LEE F. HAWLEY, OF MADISON, WISCONSIN, ASSIGNOR TO THE UNITED STATES OF AMERICA.

## PROCESS FOR PRODUCING DENSE CHARCOAL.

1,369,428.

Specification of Letters Patent. Patented Feb. 22, 1921.

Application filed April 3, 1919. Serial No. 287,316.

*To all whom it may concern:*

Be it known that I, LEE F. HAWLEY, a citizen of the United States, residing at Madison, in the county of Dane and State of 5 Wisconsin, have invented certain new and useful Improvements in Processes for Producing Dense Charcoal, of which the following is a specification.

This invention relates to an improved 10 process and apparatus for making a very dense and homogeneous charcoal from wood or similar vegetable material.

Ordinarily, the distillation of wood in the manufacture of charcoal has provided a 15 light porous charcoal. The density of the resultant charcoal has always varied with the type of wood used, a very heavy dense wood providing a charcoal normally more dense than that made from the lighter types 20 of wood. As a result of the present invention it is now possible to obtain from the lighter types of wood a charcoal much more dense than that heretofore obtained from the heaviest woods.

25 The present invention makes it possible to provide a charcoal having a density of at least .95 when an ordinary light wood is used, and a density of at least 1.05 when this same wood has been given a preliminary 30 hydrolyzing treatment.

The process comprises the comminution of the wood to saw-dust or wood flour and the compression of this material in molds into solid blocks. These blocks are formed under 35 a pressure of at least 30,000 pounds per square inch. The blocks thus formed are then distilled and at the same time subjected to a directly applied mechanical compression involving widely varying pressures as 40 differentiated from constantly applied pressure. By the term varying is meant a pressure increasing from fifty pounds per square inch to one hundred and twenty pounds per square inch and then decreasing through 45 the same range in successive alternations.

It has been found that an unusually dense charcoal is produced when the pressure is increased regularly from fifty to one hundred and twenty pounds followed by a 50 decrease through the same range with regularly recurring cycles of such increasing and decreasing pressure. Such pressure on the briquets during distillation will vary from a minimum of fifty pounds per square inch 55 to a maximum of one hundred and twenty

pounds per square inch through regular recurring cycles. This remarkable result is effected by the mechanical compression during distillation and is due in part to the fact that there is a stage in the distillation of 60 the blocks of compressed wood, just as the wood is decomposing into charcoal, when the charcoal is slightly plastic and a sufficiently great pressure therefore closes the pores and interstices thereof and forms a 65 homogeneous dense charcoal. One other reason for the remarkable results obtained is that during the period of low pressure the vapors generated by distillation are allowed to escape freely from the briquets, whereas 70 during the periods of high compression the pores of the charcoal are closed and the vapors and gases cannot escape.

The detailed steps in the process may be carried out as described hereinafter. Any 75 ordinary wood, such as birch, maple, or pine is cut or ground to a finely divided condition like saw-dust or wood flour. This comminuted material is then compressed in any suitable mold, not shown, under a pressure 80 of at least fifteen tons, 30,000 pounds, to the square inch, thus forming a solid block of wood having a density of about 1.10. These blocks or briquets are preferably circular in cross section and with smooth flat ends. A 85 desirable size is one having a diameter of four inches and a thickness of three inches. The briquets so made are then placed face to face in a metal tube, having a diameter slightly greater than that of the briquets. 90 If placed face to face within the tube the briquets form a rod of compressed wood. However, if it is desired to space the briquets apart, either to permit the passage of gases or to preserve the identity of the briquets, this may be done by introducing between the briquets thin sheets of metal of the same diameter of the briquets, or smaller than the bore of the tube. Endwise pressure 95 is applied to the column of briquets. This 100 pressure is variable and is applied in cycles varying from periods using fifty pounds per square inch to periods using a hundred and twenty pounds per square inch. The tube and its contents are subjected to a distillation temperature of at least three hundred degrees C. during which treatment the pressure is varied as above described. The plastic stage of the material during distillation 105 covers only a small range of temperatures, 110

from about 280° C.—300° C., and if the distillation temperature is carried much above this point is not necessary, and often not desirable, to apply extreme pressure during 5 the last stage of distillation.

Volatile products of distillation consisting of tar, pyrolygneous acid and gases can be trapped and used as desired as in the usual distillation of wood.

- 10 The same unusual results and dense charcoal may be obtained by utilizing a hydrolyzed wood product as the material for the briquets. In the process using hydrolyzed wood the comminuted wood is 15 treated with dilute acid, preferably sulfuric acid, and high pressure steam, about 100 pounds per square inch, the water, sugar and other soluble materials are removed, the remaining material dried and 20 briquetted and distilled as before. The resulting wood products remaining after the extraction process is produced in large and commercial quantities in the manufacturing plants engaged in the manufacture of ethyl 25 alcohol from waste wood. If this residue is briquetted and distilled under the conditions of this invention the resultant charcoal is denser, about 1.05, than that obtained directly from wood by the process.

The process may be conducted in any suitable form of apparatus capable of performing the steps specified. The briquets may be formed in any suitable machine. The 35 combined distillation and variable compression steps require an unusual type of apparatus, a suitable form of which is provided for by the present invention, which form is illustrated in the accompanying drawing, in which—

40 Figure 1 is a vertical sectional elevation illustrating the compression tube mounted in the distilling chamber,

Fig. 2 is a sectional view taken on the line 2—2 of Fig. 1,

45 Fig. 3 is a view taken on the line 3—3 of Fig. 1 looking in the direction of the arrow, and

50 Fig. 4 illustrates diagrammatically the arrangement of contacts and circuits for effecting the variable pressure feature.

Referring in detail to the drawing 1 indicates the masonry of the end walls of a distillation furnace, 2 indicates the side walls and 3 the top of the furnace. The 55 necessary strength for the structure is made certain by the liberal use of metal reinforcing where necessary. Each of the end walls has two parallel I-beams 4 positioned vertically and mounted in a concrete base 5.

60 Suitable braces 6 are provided to strengthen the lower ends of the beams 4 and tie-rods 7 extend from the upper part of the beams 4 to further brace the structure. The furnace is long and narrow and is adapted to 65 be heated by any type of fuel. As illus-

trated, the furnace is constructed to use gas or oil as fuel. Adjacent the lower part of the side walls 2 and spaced along the sides of the same are a series of ports or openings 8 adapted to receive burner nozzles projecting from any suitable supply gas pipe or oil pipe. The flame and hot gases pass upward and through the outlet openings 9 provided in the top 3.

The apparatus for compressing the briquets during distillation includes a cylindrical metal tube or pipe 10 extending longitudinally of the furnace and projecting beyond the end walls thereof. This pipe 10 is necessarily of heavy metal and in order to conform with the preferred type of briquet should have a 5 inch bore. The pipe 10 is positioned and securely held in one end wall 1 by the facing clamps 11 which are screw threaded on the pipe 10 and 80 which clamp the wall and I-beams. The opposite end of the pipe 100 is securely positioned in the opposite end wall but is not clamped to the wall, thus allowing for longitudinal movement resulting from expansion or contraction of the tube during heating. Briquets are inserted into the bore of the pipe 10 through the end opening 12 which is provided with a cover plate 13 adapted to be bolted in place over the end 85 of the pipe 10. Gases and vapors generated during the distillation pass upward and outwardly through the gas outlet passage 14 which is located between the cover plate 13 and the end of the furnace. Compression is 90 effected by means of a plunger 15 having a drive rod 16 projecting beyond the packing gland 17 and extending to drive means 95 as indicated by the worm drive 18. A motor 19 is provided to operate the worm drive 18 by connection through a chain or belt 20. The mechanism for effecting the variable compression, hereinbefore described, will be understood from the following description. The drive rod 16 is formed in two parts 100 and the adjacent ends are provided with guide plates 16<sup>a</sup> and 16<sup>b</sup> having rollers 21 adapted to engage the guide rails 22 which are positioned parallel to the rod 16 and thus adapted to prevent the vertical or lateral 105 buckling of the ends of the rod 16. The plates 16<sup>a</sup> and 16<sup>b</sup> have countersunk seats 23<sup>a</sup> and 23<sup>b</sup> adapted to receive the compression spring 24 which latter is designed and so calibrated that the pressure is known for 110 required changes in spring length. The compression of the spring 24 for a certain measured distance, therefore, will correspond with a certain definite pressure. Mounted on the adjacent faces of the plates 16<sup>a</sup> and 16<sup>b</sup> 115 are insulating blocks 25 and brackets 26<sup>a</sup> and 26<sup>b</sup> are secured to these blocks. A contact arm 27 is pivotally connected to bracket 26<sup>a</sup> and is positioned to make electrical contact alternately with the adjustable contacts 120 125 130

- 28<sup>a</sup> and 28<sup>b</sup> which latter are insulated from each other and from their respective supports 16<sup>a</sup> and 16<sup>b</sup>. For example, 28<sup>a</sup> and 28<sup>b</sup> may be set so that when the pressure 5 on the spring 24 is 120 pounds, 27 touches 28<sup>a</sup> and when the pressure drops to 50 pounds 27 will be in contact with 28<sup>b</sup>. A contact between 27 and 28<sup>b</sup> will start the driving motor 19 by energizing a solenoid 10 29 and thus drawing in rocker arm 30 closing the switch 31 and completing the circuit through the motor 19. A contact between 27 and 28<sup>a</sup> will energize the solenoid 32 and operate to draw in the rocker arm 30 15 and open the switch 31 and thus open the motor circuit. By adjusting 28<sup>a</sup> and 28<sup>b</sup> it is therefore possible to obtain any range of pressure desired throughout the distillation. If 28<sup>a</sup> and 28<sup>b</sup> are very close together, a 20 practically constant pressure is maintained, but if 28<sup>a</sup> and 28<sup>b</sup> are adjusted some distance apart, the pressure is constantly varying throughout the distillation process. It has been found that with pressures varying 25 from 50 pounds to 120 pounds, the quality of the charcoal is very much better than in the case where the limits of pressure are, for instance only 80 pounds to 100 pounds, which latter variation is substantially just enough 30 to give a satisfactory operation of the make-and-break control mechanism. The movement of the plunger 15 is reciprocatory and is provided for by an interrupted drive rod making it possible to avoid rotary movement 35 of the plunger.
- The invention described and claimed in the copending application Serial Number 287,315 provides for a change in the nature of the material treated by the use of certain 40 details of the process and certain pressures applied during distillation. The present invention is particularly directed toward the manner of applying variable pressure during distillation.
- 45 What I claim is:
1. The process of making charcoal having a specific gravity of at least .95 from wood which comprises comminuting wood, forming blocks of the comminuted wood, subjecting the blocks to pressure of at least 50 30,000 pounds to the square inch, and distilling the blocks under a directly applied mechanical pressure increasing from 50 pounds per square inch to 120 pounds per square inch and then decreasing through the same range in successive alternations.
2. The process of making a dense and homogeneous charcoal which comprises forming blocks by compressing comminuted wood, subjecting the blocks to a pressure of at least 30,000 pounds per square inch prior to distillation, and subjecting the blocks to a combined distilling temperature and to a directly applied mechanical pressure increasing from 50 pounds per square inch to 120 pounds per square inch and then decreasing through the same range in successive alternations.
3. The process of making charcoal having a specific gravity of at least .95 which comprises forming blocks by compressing comminuted wood, subjecting the blocks to a pressure of at least 30,000 pounds per square inch prior to heating them, subjecting the blocks to a combined heat treatment of 300° C. and to a directly applied mechanical pressure increasing from 50 pounds per square inch to 120 pounds per square inch and then decreasing through the same range in successive alternations.
4. The process of making charcoal having a specific gravity of at least .95 from wood, which process comprises comminuting wood, forming blocks of the comminuted wood, subjecting the blocks to mechanical pressure to compress the same, and distilling the blocks under directly applied mechanical pressure increasing from low pressure to high pressure and then decreasing from high pressure to low pressure in successive alternations.
5. The process of making a dense homogeneous charcoal which process comprises treating blocks of woody material to a combined distilling temperature and to a directly applied recurrent mechanical pressure always greater than atmospheric pressure and increasing and decreasing through the same range of pressure in successive alternations.
- In testimony whereof I have affixed my signature.

LEE F. HAWLEY.